

Oct. 21, 1924.

1,512,286

C. A. HORTON

METHOD OF MAKING CURVED FABRICS

Filed June 17, 1922

*Fig. 1.*



*Fig. 2.*



*Fig. 3.*



*Fig. 4.*



*Fig. 5.*



Charles A. Horton

By *Masou Fenwick Lawrence*,  
Attorneys

## UNITED STATES PATENT OFFICE.

CHARLES A. HORTON, OF PROVIDENCE, RHODE ISLAND, ASSIGNEE TO HOPE WEBBING COMPANY, OF PAWTUCKET, RHODE ISLAND, A CORPORATION OF MASSACHUSETTS.

## METHOD OF MAKING CURVED FABRICS.

Application filed June 17, 1922. Serial No. 569,015.

To all whom it may concern:

Be it known that I, CHARLES A. HORTON, a citizen of the United States, residing at Providence, in the county of Providence and State of Rhode Island, have invented certain new and useful Improvements in Methods of Making Curved Fabrics; and I do hereby declare the following to be a full, clear, and exact description of the invention, such as will enable others skilled in the art to which it appertains to make and use the same.

This invention relates to fabrics and more particularly to the manufacture of cloth in which threads or yarns of one or both systems or series of which it is composed curve in the plane of the fabric when laid flat.

For some purposes it is desirable to produce a woven fabric in which some, or all, or either or both systems of interlaced yarns or threads, curve in the plane of the fabric. Cloth having either the warp or filling extending in curved lines (when the cloth is in a flat state) are useful in making articles such as folded collars, either of one or of more than one piece, since, in order to make a collar of good fit, as is well known, it is necessary that the fold line be curvilinear,—that is, when the collar is flattened out. It is apparent that a folding collar, made integral of one piece of cloth, can be more readily folded on a curvilinear fold-line when one system of threads of the fabric of which it is made is similarly curved and runs parallel to the fold-line; also that a two piece cloth collar having the edges of the neck band and outer panel stitched together along the fold is better and more easily made if the threads of one system run parallel to the fold than if both systems or series of threads (the warp and weft, or filling) cross the fold line and have to be severed in cutting the pieces to the necessary curve. In order that the outer panel of two piece, folded, or turn-over collars may set off from the neck band so that the tie will slip or render easily and not bind between the outer panel and the neck band, they are usually made with the outer panel a little longer than the inner panel and the edges are brought to the same length when stitched together, thus producing an

offsetting of the outer panel from the neck band that affords room for the tie. In fabrics, woven on a curve, from which to manufacture one piece collars, the offset effect is produced by the greater length of longitudinal threads in the outer panel, as compared with the length of longitudinal threads in the inner panel, or neck band portion, to the same number of cross threads. Curved fabrics of the described character are also useful in making bands or belts, folded or unfolded, constructed to encircle a body of greater diameter at one part thereof than at another part encircled by the band, as for example, in waist or other bands designed to surround tapering parts of the human body.

Fabrics, the warp threads of which curve in the plane thereof, have been heretofore woven on narrow ware or webbing looms. Patent to Morgan, Number 1,254,340, dated January 22, 1918, discloses how webbing or other narrow fabrics may be curved in weaving. An ordinary webbing loom may be adapted to produce webbing with a curvilinear warp by equipping it with a set of conical take up rolls and a conical or inclined guide on the edge of the breast beam for each piece of webbing being woven, and also with an additional number of warp beams in order to cause the warp yarns or threads that are woven into the fabric adjacent the convexed outer edge to feed faster than those that are woven into the fabric adjacent the concaved edge. In a webbing loom operating, say twenty to thirty shuttles, the expense of installation of the necessary additional warp beams, conical feed rollers and special guides, greatly increases the loom cost as compared with the original cost of looms fitted to weave straight webbing. Furthermore, the stretching to which a large proportion of the warp threads must be subjected in order to be properly woven into a curved fabric results in more frequent breakage of these threads and more frequent stoppage of the loom, in order to tie in the broken warp ends, than is the case when weaving straight webbing with equal feed of warp threads. The cost of production of webbing curved in the weaving process, it will be apparent, is much higher than the cost of straight warp webbing of the

same dimension, weave, weight and quality of yarn.

By my invention I am able to produce woven strips curved in the plane of the fabric, or of different widths in different portions, on either narrow ware or broad cloth looms, by weaving them with straight filling and uniformly fed warp, and thereafter imparting a desired curvature or other predetermined modification of form by the usual washing, bleaching, dyeing or like finishing operations. And the invention consists: of a fabric having adjacent areas or zones possessing relatively different shrinkage capacities; of a method of producing fabrics curved in the plane thereof which consists in weaving a fabric with substantially equal feed of warp and straight intersecting filling, adjacent areas or zones of the fabric having different relative shrinking capacities, then uniformly moistening the fabric, thereby causing the different zones to shrink unequally. It further consists in the combination of structural details and specific combination of steps described and claimed hereinafter.

In practicing this invention no process additional to the finishing operations to which woven fabrics are usually subjected is necessary, because the customary bleaching, dyeing, washing or shrinking treatment imparts a new form to cloth made in accordance with the invention. For example, cotton fabrics woven of the natural cotton yarn, when delivered from the loom are of a creamy shade and may be slightly soiled in the process of manufacture, and it is customary to treat these goods with bleaching liquids if white cloth is required. The usual bleaching and finishing operation imparts the degree of re-formation which the fabric has been particularly designed to have by reason of the different structure of the thread systems in different areas, or the different kinds of fiber, or both.

In the accompanying drawings which illustrate the invention diagrammatically:

Figure 1 is a plan view of a piece of straight woven webbing having adjacent longitudinal areas or zones one of which has the capacity of shrinking or contracting longitudinally more than the other after uniform moistening;

Figure 2 is a plan view of the same piece of webbing after having been moistened, as in the bleaching operation;

Figure 3 is a diagrammatic cross section assumed to have been taken on the line 3—3 of Fig. 1;

Figure 4 represents, in full lines, a piece of straight webbing having three longitudinal areas or zones of different shrinkage capacity, and in dotted lines the same piece of webbing after having been bleached or otherwise moistened; and

Figure 5 is a diagrammatic cross section assumed to have been taken on the line 5—5 of Fig. 4.

The diagrammatic illustrations are merely exemplary of fabric structures embodying this invention. Different relative shrinkage capacities,—that is, capability of contracting, when moistened, different percentages,—may be imparted to adjacent longitudinal areas or zones by many different expedients without departing from the principle of this invention. The weft or filling of the fabric illustrated is of the same count (size) and has the same number of picks to the inch throughout a given web. But, variations are shown in the warp, whereby to provide known and definitely controllable differences of percentage of shrinkage in the direction of the warp in different longitudinal areas, zones or panels. The relative shrinkage capacities of the warp yarns may be varied progressively from one selvage edge to the other, or they may be varied progressively in groups, zones or bands; and, furthermore, the radius of curvature imparted to the fabric after moistening or bleaching may be predetermined with accuracy. It is not practicable to illustrate all of the expedients by which different relative shrinkage capacities may be imparted to different longitudinal areas. Different degrees of capacity to contract may be imparted to adjacent zones by using fiber of different kinds for the warp threads of the different zones; or by variations in the warp structure; or both. Warp structure may be varied in many ways to achieve the desired result; the warp threads of one zone may be of a different count than those of another; they may be composed of multiply strands twisted together with a different number of turns to the inch, or one zone may be provided with straight stuffing warp threads that are absent in another zone or are more numerous in one zone than in another, or other differences of structure may be introduced in different areas to produce the desired effect. Similar variations in the filling threads may be utilized to produce cloth susceptible of assuming a precalculated non-rectangular outline, and combinations of both warp and filling, varied as described, may be adopted for the purpose of producing cloth and cloth articles of predetermined form, as will be apprehended by persons skilled in textile arts.

It is to be understood, therefore, that the invention is not dependent upon any particular means whereby one area or zone of cloth is caused to shrink a greater or less percentage than another.

In Fig. 1 is conventionally illustrated a piece of unbleached, straight woven webbing, said webbing having two panels, 1 and 2, joined by a narrow zone 3, along which

the fabric is capable of folding more easily than elsewhere, and in which panels 1 and 2 are so constructed that if the webbing is immersed in water, or any usual bleaching or 5 dyeing liquid, it will assume, after drying the form indicated conventionally in Fig. 2. Panels 1 and 2 and the fold zone 3 (of Fig. 1) have assumed a distinct curvilinear form, as indicated at 1<sup>a</sup>, 2<sup>a</sup> and 3<sup>a</sup>, (Fig. 2), the 10 warp of the inner panel 1 having contracted more than that of the outer panel 2, thus causing the narrow fabric to bend, and the straight fold zone 3 having assumed a curvilinear course corresponding to that of the 15 panels.

In Fig. 3, which is a conventional cross section on the line 3—3 of Fig. 1 there is illustrated one varying warp construction which adapts the straight fabric indicated in Fig. 1 to be converted by shrinking into the curved fabric indicated in Fig. 2. For purposes of exemplification a two ply interwoven fabric suitable for use in making folded collars is shown. The warp ends of the face ply in the panel 2, 2<sup>a</sup> and in the fold zone 3, 3<sup>a</sup>, are indicated by 4 and the filling by 5. The warp ends of the back ply of panel 2, 2<sup>a</sup> and the fold zone 3, 3<sup>a</sup> are indicated by 4<sup>a</sup> and the filling of the said back ply by 5<sup>a</sup>. Between the face and the back plies of the panel 2, 2<sup>a</sup> and of the fold zone 3, 3<sup>a</sup>, are straight stuffing warp threads 6, which may be, as shown in Fig. 3, equal in number to the warp threads of the face or back plies. The stuffing threads 6 are not interlaced in the fabric, but lie straight between the two plies. At intervals are binder threads 7, which tie the front and back plies firmly together and hold the stuffing warp 40 clamped between them. The panel 1, 1<sup>a</sup> is shown as comprising two plies bound together by binder threads, but devoid of stuffing warp, the warp of the face ply in panel 1, 1<sup>a</sup> being indicated by 14 and the warp of 45 the back ply by 14<sup>a</sup>. The same filling 5, 5<sup>a</sup> is woven in the panel 1, 1<sup>a</sup>, as in the panel 2, 2<sup>a</sup> and the fold zone 3, 3<sup>a</sup>. It will be apparent that a similar result, differing only in degree 50 may be produced by inserting relatively fewer stuffing warp threads in panel 1 than in panel 2.

Webbing of a weave conventionally illustrated in Fig. 3, when uniformly moistened and dried, assumes a curvilinear form, as 55 indicated in Fig. 2, for the reason that panel 1, if woven of yarn having the same percentage of shrinkage as panel 2, will shrink more than panel 2 by reason of the fact that the straight stuffing warp threads present in 60 panel 2 will restrain the shrinking of panel 2. In explanation it may be stated that yarn of greater length will shrink a greater absolute amount than yarn of lesser length although the percentage of shrinkage capacity 65 may be the same in both. The stuffing

warp threads in the illustrated fabric are straight and much shorter than the interlaced warp and binder threads. The actual amount of shrinkage, therefore, of which the stuffing threads in a given length of fabric are susceptible is much less than that of which the interlaced threads in the same length of fabric are susceptible. The stuffing warp being clamped firmly by the binder threads between the two plies in panel 2 70 prevent the shrinkage of panel 2 to the same extent as panel 1, which is devoid of stuffing warp and is composed entirely of interlaced and crimped threads free to shrink 75 without such restraint.

If the warp threads in the panel 1 were of the same count as the face and back warp of the panel 2, the weight of the fabric in panel 1 would be less to the square inch than in panel 2. Should it be desired to have the fabric of the same weight to the square inch throughout, the loss of weight due to omission or reduction in number of stuffing warp threads may be compensated for by the use of coarser and heavier warp thread; for example, the warp in panel 2 may be 60/2 cotton yarn and the warp in panel 1 may be 40/2 cotton yarn,—that is to say, the warp in panel 2 may be sixty count cotton yarn composed of two strands twisted together, and the warp of panel 1 may be forty count cotton yarn composed of two intertwined strands. The filling should be the same in both panels for the sake of uniformity of appearance and simplicity of weave. The appearance of the fabric constructed as indicated in Fig. 3 will be the same throughout, since the filling is the same and the difference in size of warp threads in the two panels is not noticeable.

The fabric conventionally shown in Figs. 1 to 3 will be understood to exemplify one means by which the desired result may be achieved. A like result may be achieved by other expedients some of which have heretofore been mentioned.

In Fig. 4 there is illustrated in full lines a piece of straight woven webbing (which may be narrower than that illustrated in Figs. 1 to 3) in which three parallel zones, a, b and c, are indicated, zone "b" being so constructed as to have the capacity of shrinking longitudinally more than zone "a," and zone "c" more than zone "b." The dotted curved lines indicate the form of the webbing after shrinking. It is shown as a two ply interwoven fabric provided with stuffing warp. The filling 5, 5<sup>a</sup> may be of the same type and quality of yarn throughout, for example, the filling may be 60—2 cotton yarn of eighty picks to the inch in each ply, and all warp yarns, including the stuffing warp and the binder, may be of the same count, material and structure as the filling. The difference in relative 115 120 125 130

shrinkage capacity of the different zones may be effected by varying progressively the number of stuffing warp threads to the inch, while providing the same number of face and back warp threads to the inch throughout. For example, zone "a" may have eighty stuffing warp ends to the inch, zone "b" may have sixty and zone "c" may have forty. Thus, after moistening and drying, shrinkage of zone "c" is restrained by fewer straight stuffing warp threads than zone "b," and the shrinkage of zone "b" is restrained by fewer straight stuffing warp threads than zone "a"; and, as a consequence, zone "c" will shrink more than zone "b," and zone "b" more than zone "a," thus imparting the curvature indicated. It will be obvious that the radius of curvature to be obtained may be varied by varying the number of stuffing warp yarns in the several zones or by omitting them from the zone to be shrunk the most.

It will be apparent to those skilled in the art of cloth finishing and familiar with the properties of textile fibers that the principles of this invention may be applied in many other ways than those illustrated and specifically described.

Utilization of fabric having different shrinkage capacities in different parallel areas or zones, when it is desired to produce a fabric curved in the direction of one system of interlaced threads, enables a fabric so curved to be obtained at a cost no higher than that of production of straight fabric, since the curvature may be imparted in the shrinking, bleaching or dyeing process to which fabrics are commonly subjected before use. In the manufacture of collars it is assumed that the collars may be die-cut from the fabric shown in Fig. 2, the neck band being cut from panel 1<sup>a</sup> and the outer fold portion from the panel 2<sup>a</sup>, so that the collar may fold along zone 3<sup>a</sup>. If two piece collars are desired the neck band and the fold portion may be separately cut from narrow webbing such as is indicated in Fig. 4, the convex selvage edge of one piece lapped over the concave edge of the other and the two parts stitched together, the overlapping portion of the neck band portion constituting a fold guide, along which the collar may be folded.

The principle of making fabric adapted to be curved by different longitudinal shrinking of adjacent areas in the bleaching and finishing operation may be carried out in the manufacture of broad cloth as well as in the manufacture of narrow ware and webbing. Broad cloth may be woven on a fly shuttle loom in a plurality of connected bands or relatively narrow areas, of the character exemplified in Fig. 1, or in Fig. 4, and the lines of demarkation between them indicated by any suitable expedient such as

by inserting a colored warp thread between them or omitting one or several warp threads. The broad fabric may then be cut along the demarkation line and the bands or strips thus severed treated at the 70 bleachery.

Besides the economies referred to in producing curved fabrics by this method, there is a distinct advantage in handling straight fabric at the bleachery as compared with 75 the handling of curved fabric, for the reason that the straight fabric is better adapted to be wound on a roll or spool and to feed therefrom.

As has been pointed out, the fabric is 80 straight woven. In all weaving operations, the yarns are customarily and necessarily, under the present state of the weaving art, set in the looms under considerable tension, and this tension necessarily tends to 85 stretch the yarns. When the tension is removed, there is necessarily a counter-action of contraction. When the fabric is of substantially the same construction throughout, the shrinkage or contraction in the fabric after it has been taken from the loom is substantially the same throughout the fabric which therefore remains substantially straight as it was woven. When, however, the fabric is made in accordance with the 95 present invention, that is to say of varying construction in adjacent panels, the natural or normal contraction of the fabric after it has been taken from the loom is such as to impart a slightly curvilinear effect to the 100 fabric. This curvilinear effect is not very pronounced in a short section of fabric but is readily discernible in a long piece and is an advantage rather than a disadvantage inasmuch as the direction of subsequent 105 curvature of the fabric is readily perceived.

The principle of this invention is applicable to single ply fabric, as well as to multiply interwoven fabrics, although in the case of single ply fabrics, stuffing yarn cannot be used in the manner described with reference to multiply fabrics. But it will be apparent that different relative shrinking capacities may be given to different areas by using yarns or threads of different twist, 110 or of different materials, or of different counts or other combinations for the purpose.

What I claim and desire to secure by Letters Patent is:—

1. Fabric having straight areas extending lengthwise thereof composed of unshrunken threads, one of which areas has the capacity of shrinking a different percentage than another whereby, when moistened, 125 curvature will be imparted to the fabric.
2. Woven fabric having straight areas extending lengthwise thereof composed of unshrunken threads, one of which areas has the capacity of shrinking a different per- 130

centage than another in the direction of the threads of that system that are parallel to the threads of the same system in the other whereby, when the fabric is moistened, curvature will be imparted to the fabric.

3. Woven fabric having straight adjacent areas extending lengthwise thereof composed of unshrunken threads, the warp threads in one of which areas are substantially parallel 10 with the warp threads of another, one of said areas having the capacity of shrinking a different percentage than another in the direction of the warp when moistened whereby curvature will be imparted to the fabric.
- 15 4. Woven fabric having adjacent areas extending lengthwise thereof composed of unshrunken threads of different shrinking capacity, that system of threads in one area which is parallel to the corresponding 20 system in the other having a difference of structure such as to impart to one area the capacity of shrinking in the direction of the threads of said system a greater percentage than the other when moistened 25 whereby curvature will be imparted to the fabric.

5. Multiply woven fabric having adjacent areas, one of which has the capacity of shrinking a different percentage than another, one system of threads in one area having a different structure than the corresponding parallel system of threads in another in that the said system of one area includes straight threads tending to restrain 30 the shrinkage thereof as compared with another.

6. The method of producing fabric which consists in forming a straight woven fabric with adjacent areas composed of unshrunken 40 threads, one area having the capacity of shrinking a different percentage than another, then moistening said fabric equally thereby causing one area to shrink a greater percentage than another.

45 7. The method of producing fabric which consists in weaving a straight web of unshrunken threads in such manner that adjacent areas have the capacity of shrinking

a different percentage in the direction of that system of threads in one that is parallel 50 with the corresponding system in another, then moistening said areas equally, thereby causing one area to shrink a greater percentage than another whereby the fabric will assume a curved form.

55 8. The method of producing fabric which consists in weaving a straight web of unshrunken threads with adjacent areas having substantially parallel warp threads, one of said areas having the capacity of shrinking 60 a greater percentage than another in the direction of the warp, then moistening said areas equally, thereby causing one area to shrink a greater percentage than another whereby the fabric will assume a curved 65 form.

9. The method of producing fabric, which consists in weaving a straight web of unshrunken threads with adjacent areas having inherently different shrinkage capacities, that system of threads in one area, 70 which is parallel to the corresponding system in another, having a different structure such as to impart to one area the capacity of shrinking in the direction of the threads 75 of said system a greater percentage than the other, then moistening said areas equally thereby causing one area to shrink a greater percentage than the other whereby the fabric will assume a curved form.

80 10. The method of producing a strip of multiply fabric curved in the plane thereof, which consists in weaving a web with adjacent zones extending longitudinally of one system of threads, said system in one zone having a different structure than in another in that said system in one zone includes straight stuffing threads tending to restrain the shrinkage of that zone as compared with another, then moistening said zones equally, 85 thereby causing one zone to shrink a greater percentage than another.

In testimony whereof I affix my signature.

CHARLES A. HORTON.